

## UNITED STATES PATENT OFFICE

2,382,632

PROCESS FOR RENDERING WOOL  
NONFELTING

Frederick A. Hessel, Montclair, and John B. Rust,  
Verona, N. J., assignors to Ellis-Foster Com-  
pany, a corporation of New Jersey

No Drawing. Application November 18, 1941,  
Serial No. 419,634

8 Claims. (Cl. 8—127.8)

This invention relates to a process of preventing the felting of wool and animal furs by treatment of the aforesaid materials with basic nitrogen compounds at elevated temperatures.

It is known that it is possible to produce non-felting and non-shrinking wool by chlorination and bromination of the material in aqueous solution. There have also been described processes of producing non-felting wools by treatment with sulfonyl chloride, chromyl chloride, nitrosyl chloride and the like. The latter processes, however, require the use of organic solvents and therefore have only limited commercial applicability. These processes are usually carried out at low temperatures, that is, at ordinary room temperature or very slightly thereabove.

The present process comprises the treatment of wool (either as the raw wool, yarn, knit or woven goods) in an aqueous bath containing from 1 to 10 per cent of a water-soluble basic nitrogen compound at temperatures usually ranging from 50° to 90° C. and at atmospheric pressure or higher depending upon the volatility of the compound. When wool is treated in this manner for periods varying from 15 minutes to 1 hour, then rinsed and dried its properties have been altered to such a degree that it no longer has a tendency to felt during washing and consequently is non-shrinking also. We have found that various types of basic nitrogen compounds are suitable for this purpose: water-soluble primary and secondary amines, compounds of analogous basic nature such as hydroxylamine, hydrazine, semicarbazide, guanidine and the like; tetraethanolammonium hydroxide, tripropanoylethanolammonium hydroxide, and other mildly basic quaternary ammonium hydroxides which do not have a dissolving action on the wool; alkali salts of amino acids such as sodium aminoacetate and the salts of the amino acids of proteins. Ammonium carbonate is moderately effective but shows best results when used in combination with one of the other nitrogen compounds.

Usually if wool is heated for any extended length of time in water under alkaline conditions at 50°-90° C. it has a tendency to felt badly and, therefore, it is surprising that under the conditions of the present invention, just the reverse is true and excellent non-felting characteristics are imparted to the wool by this treatment.

The method used for testing the non-felting characteristics imparted to wool by the present

process involves a series of washings. The treated wool is placed in a large volume of hot (90°-100° C.) water containing ½% of neutral soap in a washing machine and worked for 1 hour, after which the wool is rinsed and dried. The number of such treatments which the treated wool can endure before definite signs of felting are noted is taken as a measure of its resistance to felting. This washing procedure is similar to that used to test the permanency of cotton finishes and may be considered as quite drastic for wool.

Certain of the chemicals used herein (particularly when the treatment is too pronounced) may cause yellowing of the fiber. Where this coloration is not desired it may usually be removed by a light bleaching treatment. Wetting agents improve the uniformity of the treatment. The feel of the goods is usually unaltered but in certain cases a slight harshness may be encountered, which can be overcome by softening agents.

The alkalinity of the treating bath is in general about pH 11 but this may vary in certain cases between about pH 8 and pH 12. The temperature which has been found most satisfactory is about 75° C. for about one half hour. However, as mentioned previously, a temperature in the general range of about 50° to 90° C. and, correspondingly, for from 60 minutes for the lower temperature to 15 minutes for the higher range is suitable. Other materials may also be present in the treating bath to accelerate or mitigate the reactions involved between the amine and wool. Such materials may include sodium sulfate, sodium chloride, sodium acetate, sulfonated oils or long chain substituted aromatic derivatives, wetting agents such as sodium lauryl sulfate, dioctyl sodium sulfosuccinate and the like.

Furthermore, since the present process is carried out under alkaline conditions we have found that it may be combined with certain operations normally used in wool processing such as the preliminary and final scouring steps. For instance, wool knit goods was entered in a bath containing 2% of a sulfonated fatty oil derivative (e. g., that material sold under the name of Sulfanole) and 4% of a basic nitrogen compound (e. g., monoethanolamine) at 75° C. The treatment was continued for 40 minutes, then the wool was rinsed thoroughly and dried. By this treatment the wool was thoroughly scoured and had acquired non-felting qualities as shown by the series of washings described above.

Example 1.—As a specific embodiment of the present invention a piece of undyed knitted wool measuring 4 cm. x 4 cm. and weighing 6.9 grams was immersed at 70-75° C. for 30 minutes in a solution containing 4 g. isopropylamine in 96 g. water. The solution at the start and at the end of the treatment had pH 11. Following this treatment the sample was rinsed thoroughly with cold water and dried. Color and feel of the piece were unchanged. The effectiveness of the process in preventing felting was determined by a series of washings in hot water as mentioned above. The sample withstood eight washings without felting and retained its original dimensions.

A similar knitted sample immersed in water at 75° C. for 30 minutes did not withstand 2 washings, but felted and had shrunk badly. The same was true of knitted wool which was merely washed.

By way of other illustrative examples, there is

presented below a table showing the results of tests with a large number of basic nitrogen compounds. The compounds were dissolved in water at various temperatures in the amount shown. The pH of each solution was determined by indicator papers. Pieces of wool knit goods were immersed for the indicated period (time in hours), and after this simple immersion treatment the wool pieces were rinsed thoroughly with cold water and dried. Color (if any) imparted by the treatment and also the feel of the dried goods is noted. Thereafter the pieces were washed as described above and the number of washings which the wool was able to withstand before evidences of felting were noticed in the dried piece is recorded as a measure of felt-resistance resulting from the treatment. It may be remarked that, according to our observations, untreated wool will stand from 1 to 2 of the standard washings.

| Example | Nitrogen compound                                                                   | pH | Temper-<br>ature,<br>°C. | Time,<br>hours | Color           | Feel           | Number<br>washings<br>before<br>felting |
|---------|-------------------------------------------------------------------------------------|----|--------------------------|----------------|-----------------|----------------|-----------------------------------------|
| 2       | 10% ethylene diamine                                                                | 11 | 20                       | 1/2            | Light yellow    | O. K.          | 2                                       |
| 3       | 4% ethylene diamine                                                                 | 11 | 65                       | 1/2            | do              | O. K.          | 6+                                      |
| 4       | 4% ethylene diamine                                                                 | 11 | 75                       | 1/2            | O. K.           | O. K.          | 1                                       |
| 5       | 4% ethylene diamine                                                                 | 11 | 75                       | 1/2            | Light yellow    | O. K.          | 4                                       |
| 6       | 4% ethylene diamine                                                                 | 11 | 75                       | 1/2            | do              | O. K.          | 7+                                      |
| 7       | 6% ethylene diamine                                                                 | 11 | 75                       | 1/2            | do              | O. K.          | 4+                                      |
| 8       | 4% ethylene diamine                                                                 | 11 | 75                       | 1              | do              | Slightly harsh | 15                                      |
| 9       | 1% ethylene diamine                                                                 | 11 | 75                       | 1              | do              | O. K.          | 1                                       |
| 10      | 1% ethylene diamine                                                                 | 11 | 75                       | 1/2            | do              | O. K.          | 10                                      |
| 11      | 1% ammonium carbonate                                                               | 11 | 75                       | 1/2            | O. K.           | O. K.          | 8                                       |
| 12      | 1% ammonium carbonate                                                               | 10 | 75                       | 1/2            | Slightly yellow | O. K.          | 4                                       |
| 13      | 1% guanidine carbonate                                                              | 11 | 20                       | 1/2            | O. K.           | O. K.          | 2                                       |
| 14      | 1% guanidine carbonate                                                              | 11 | 75                       | 1/2            | Light yellow    | O. K.          | 5                                       |
| 15      | 1% guanidine carbonate                                                              | 11 | 75                       | 1/2            | do              | O. K.          | 2                                       |
| 16      | 1% guanidine carbonate                                                              | 11 | 75                       | 1              | Brownish        | O. K.          | 10                                      |
| 17      | 1% sulfonated oil                                                                   | 11 | 75                       | 1              | O. K.           | O. K.          | 9+                                      |
| 18      | 1% tetraethanol ammonium hydroxide                                                  | 11 | 75                       | 1/2            | Yellowish       | Slightly harsh | 9                                       |
| 19      | 1% tetraethanol ammonium hydroxide                                                  | 11 | 65                       | 1/2            | do              | do             | 8                                       |
| 20      | 1% tetraethanol ammonium hydroxide                                                  | 11 | 75                       | 1              | Light brown     | O. K.          | 6+                                      |
| 21      | (2.6% tetraethanol ammonium hydroxide                                               | 11 | 75                       | 1              | do              | O. K.          | 6+                                      |
| 22      | 13.3% sodium sulfate                                                                | 8  | 75                       | 1              | do              | O. K.          | 2                                       |
| 23      | 1% tetraethanol ammonium hydroxide<br>(H <sub>3</sub> PO <sub>4</sub> to adjust pH) | 11 | 75                       | 1              | do              | O. K.          | 5+                                      |
| 24      | 1% tetraethanol ammonium hydroxide                                                  | 11 | 75                       | 1              | Light yellow    | O. K.          | 3                                       |
| 25      | 1% monoethanolamine                                                                 | 11 | 20                       | 1              | Brownish        | Slightly harsh | 1                                       |
| 26      | 1% monoethanolamine                                                                 | 11 | 75                       | 1/2            | O. K.           | O. K.          | 1                                       |
| 27      | 1% monoethanolamine                                                                 | 11 | 65                       | 1/2            | O. K.           | O. K.          | 1-                                      |
| 28      | 1% monoethanolamine                                                                 | 11 | 65                       | 1/2            | O. K.           | O. K.          | 5                                       |
| 29      | 1% monoethanolamine                                                                 | 11 | 75                       | 1/2            | O. K.           | O. K.          | 4                                       |
| 30      | 1% monoethanolamine                                                                 | 11 | 75                       | 1              | Light yellow    | O. K.          | 9+                                      |
| 31      | 1% monoethanolamine                                                                 | 11 | 75                       | 1              | do              | O. K.          | 9+                                      |
| 32      | 1% sulfonated oil                                                                   | 11 | 75                       | 1/2            | Yellowish       | O. K.          | 6+                                      |
| 33      | 2% ethylamine                                                                       | 12 | 75                       | 1/2            | do              | Slightly harsh | 9                                       |
| 34      | 2% ethylamine                                                                       | 11 | 75                       | 1/2            | do              | do             | 8+                                      |
| 35      | 2% ammonium carbonate                                                               | 11 | 75                       | 1/2            | O. K.           | O. K.          | 9                                       |
| 36      | 2% ammonium carbonate                                                               | 9  | 90                       | 1/2            | Slightly yellow | O. K.          | 8+                                      |
| 37      | 2% ammonium carbonate                                                               | 9  | 90                       | 1/2            | O. K.           | O. K.          | 8+                                      |
| 38      | 2% diethanolamine                                                                   | 11 | 75                       | 1              | Light yellow    | O. K.          | 4                                       |
| 39      | 4% 2-amino-2-methyl-1,3-propanediol                                                 | 11 | 75                       | 1/2            | Slightly yellow | O. K.          | 4                                       |
| 40      | 4% n-butylamine                                                                     | 11 | 75                       | 1/2            | Yellow          | Slightly harsh | 9                                       |
| 41      | 4% sec.-butylamine                                                                  | 11 | 75                       | 1/2            | Slightly yellow | do             | 5+                                      |
| 42      | 4% trimethylolamino methane                                                         | 11 | 75                       | 1/2            | O. K.           | O. K.          | 2                                       |
| 43      | 4% n-aminylaniline                                                                  | 11 | 75                       | 1/2            | Slightly yellow | O. K.          | 10+                                     |
| 44      | 4% 2-ethyl-butylamine                                                               | 11 | 75                       | 1/2            | do              | Slightly harsh | 10+                                     |
| 45      | 4% 2-ethyl-hexylamine                                                               | 11 | 75                       | 1/2            | O. K.           | O. K.          | 5+                                      |
| 46      | 4% diethylenetriamine                                                               | 11 | 75                       | 1/2            | Greenish cast   | O. K.          | 5+                                      |
| 47      | 4% tetraethylammonium pentamine                                                     | 11 | 75                       | 1              | Yellowish       | O. K.          | 10                                      |
| 48      | 4% morpholine                                                                       | 11 | 75                       | 1/2            | O. K.           | O. K.          | 3                                       |
| 49      | 4% benzylamine                                                                      | 11 | 75                       | 1/2            | O. K.           | O. K.          | 10+                                     |
| 50      | 4% aniline                                                                          | 8  | 75                       | 1              | O. K.           | O. K.          | 3                                       |
| 51      | 2% hydroxylamine sulfate                                                            | 9  | 65                       | 1/2            | O. K.           | O. K.          | 6+                                      |
| 52      | 2% borax                                                                            | 9  | 65                       | 1/2            | O. K.           | O. K.          | 6+                                      |
| 53      | 2% sodium carbonate                                                                 | 9  | 75                       | 1              | O. K.           | O. K.          | 8                                       |
| 54      | 2% hydrazine sulfate                                                                | 9  | 75                       | 1              | O. K.           | O. K.          | 6                                       |
| 55      | 2% monostreptidine                                                                  | 8  | 75                       | 1/2            | O. K.           | O. K.          | 2                                       |
| 56      | 2% semicarbazide hydrochloride                                                      | 12 | 75                       | 1/2            | O. K.           | O. K.          | 2                                       |
| 57      | 1.3% ammonium hydroxide                                                             | 9  | 75                       | 1/2            | O. K.           | O. K.          | 2                                       |
| 58      | 4% tributylamine                                                                    | 11 | 75                       | 1/2            | O. K.           | O. K.          | 2                                       |
| 59      | 4% triethanolamine                                                                  | 11 | 75                       | 1/2            | O. K.           | O. K.          | 2                                       |
| 60      | 2.6% aminoacetic acid                                                               | 11 | 75                       | 1/2            | O. K.           | O. K.          | 6+                                      |
| 61      | 1.4% sodium hydroxide                                                               | 11 | 75                       | 1/2            | O. K.           | O. K.          | 6+                                      |

The following examples make use of the alkali salts of protein break-down products obtained by enzymic action.

*Example 58.*—One gram of papain concentrate (proteolytic activity 10 mg.-15 seconds by Ballis and Hoover method) was added to 7.5 g. gelatin in 96 cc. water and brought to pH 5 by means of sodium sulfite. After standing for 2 days the odorless liquid was treated with sodium carbonate to pH 11, heated to 75° C. and knitted wool (1.85 g.) immersed therein for 1/2 hour. The fabric was thereafter rinsed in cold water and dried. Color and feel of the goods were satisfactory and 8 washings produced no felting.

*Example 59.*—A mixture of 7.5 g. gelatin and 0.05 g. trypsin in 100 cc. water was brought to pH 9 and allowed to stand for 3 days. During this time a white precipitate formed. The suspension was shaken up, brought to pH 10 with sodium carbonate and heated to 75° C. A piece of knitted wool (1.8 g.) was immersed for 1/2 hour, then washed and dried. Color and feel were good. Some felting was observable after 9 washings.

*Example 60.*—Four grams of glue and 0.1 g. trypsin were added to 96 g. water and the solution brought to pH 9 with sodium carbonate. After standing for 4 days the solution, which had a strong odor, was heated to 70° C. and a sample of knitted wool immersed therein for 1/2 hour. After rinsing and drying the piece showed good color and feel. It withstood 9 washings without felting.

Casein was used in place of glue in the above example with similar results.

In Examples 36 and 37 sodium formaldehyde sulfoxylate is used with ammonium carbonate. It is believed that the following reactions occur and that methyl amine is formed:



It may be remarked that under certain conditions we may operate our process at room temperature. However, the long time required makes such a temperature impractical so that we prefer, as mentioned previously, to use a temperature in the range of 50° to 90° C.

We claim:

1. Process of producing non-felting wool which comprises heating wool in an aqueous solution of from about 1-10% of a basic nitrogen compound selected from the group consisting of primary and secondary amines, mild quaternary ammonium bases which do not dissolve wool, and alkalisalts of amino acids, at 50° to 90° C. for 15 to 60 minutes; and thereafter rinsing and drying.
2. Process of producing non-felting wool which comprises heating wool in an aqueous solution of from about 1-10% of isopropyl amine at 50° to 90° C. for 15 to 60 minutes, and thereafter rinsing and drying.
3. Process of producing non-felting wool which comprises heating wool in an aqueous solution of from about 1-10% of guanidine at 50° to 90° C. for 15 to 60 minutes, and thereafter rinsing and drying.
4. Process of producing non-felting wool which comprises heating wool in an aqueous solution of from about 1-10% of ethylenediamine at 50° to 90° C. for 15 to 60 minutes, and thereafter rinsing and drying.
5. Process of producing non-felting wool which comprises heating wool in an aqueous solution of from about 1-10% of a primary amine at 50° to 90° C. for 15 to 60 minutes, and thereafter rinsing and drying.
6. Process of producing non-felting wool which comprises heating wool in an aqueous solution of from about 1-10% of a primary amine with ammonium carbonate at 50° to 90° C. for 15 to 60 minutes, and thereafter rinsing and drying.
7. Process of producing non-felting wool which comprises heating wool in an aqueous solution of from about 1-10% of isopropyl amine with ammonium carbonate at 50° to 90° C. for 15 to 60 minutes, and thereafter rinsing and drying.
8. Process of producing non-felting wool which comprises heating wool in an aqueous solution of from about 1-10% of ethylenediamine with ammonium carbonate at 50° to 90° C. for 15 to 60 minutes, and thereafter rinsing and drying.

FREDERICK A. HESSEL.  
JOHN B. RUST.